

## UNITED STATES PATENT OFFICE

2,369,149

## LUBRICANTS

Eugene Lieber, West New Brighton, Staten Island, N. Y., and Aloysius F. Cashman, Bayonne, N. J., assignors to Standard Oil Development Company, a corporation of Delaware

No Drawing. Application December 31, 1941,  
Serial No. 425,126

3 Claims. (Cl. 252—48)

This invention relates to the field of lubricants and more particularly to stabilized extreme pressure lubricants.

It is known that plain mineral oils do not have a sufficiently high film strength for lubricating moving metal parts which contact each other under high pressures, such as certain types of bearings, engines, gears, etc. It is also known that the film strength or load-carrying capacity of such mineral oils can be greatly increased by adding thereto various chemical compounds or materials containing active halogen and/or sulfur, and sometimes phosphorus, but these various materials, although very effective in carrying the high loads demanded of extreme pressure lubricants, have a serious disadvantage that during storage, especially in contact with certain metals such as iron, they undergo some type of degradation or change which tends to make certain constituents thereof insoluble and precipitate out.

It has now been found that the addition of small amounts of certain types of materials to the extreme pressure lubricating agents or to the lubricants in which they are compounded, will stabilize them against such tendencies to form an insoluble precipitate or sediment. With this primary object in view, another object of the invention is to accomplish this desired stabilization without interfering or materially reducing the extreme pressure lubricating characteristics of the lubricant and without materially increasing the corrosive tendencies of such lubricants toward metals in which they come in contact.

Broadly, the invention comprises adding to such extreme pressure lubricants from which an insoluble precipitate or sediment tends to settle out during storage, a small amount of a stabilizer comprising a high molecular weight condensation product of an aromatic compound and a condensable aliphatic compound having more than 10 carbon atoms. Such compounds are preferably made by Friedel-Crafts condensation of an aromatic hydrocarbon or various derivatives thereof such as those containing low molecular weight alkyl groups such as methyl, ethyl, etc., or other constituents such as hydroxyl groups,

etc., with a relatively long chain aliphatic compound containing a reactive group such as a replaceable halogen atom or an olefinic linkage, as for instance, chlorinated paraffin wax, or olefins derived therefrom by simple removal of hydrogen chloride without substantial cracking of the carbon-to-carbon linkages. Several such materials are available on the market. One, marketed under the trade name "Paraflo," and hereinafter referred to as stabilizer A, is made by condensing about 10-20 parts by weight of naphthalene with 90-80 parts by weight of chlorinated paraffin wax containing about 10% to 15% chlorine, in the presence of aluminum chloride as catalyst. Another material, marketed under the trade name "Santopour," hereinafter referred to as stabilizer B, is made by a similar condensation of phenol with chlorinated paraffin wax in the presence of aluminum chloride, which may or may not be further reacted upon with "acyl halides," e. g., phthalyl chloride or other resinifying agents. Most of the materials of this general class tested thus far happen to have the property of lowering the pour point of waxy mineral lubricating oils when added thereto in small amounts, for which characteristic they are frequently referred to as pour depressors, although a number of other materials which are pour depressors do not have the same type of chemical structure as these materials.

There are also a number of other materials which fall within the scope of the stabilizers of this invention. For instance, a suitable material, hereinafter referred to as stabilizer C, can be made by condensing chlorinated paraffin wax with benzene in the presence of aluminum chloride as catalyst. A still different type of material, hereinafter referred to as stabilizer D, is obtained by aluminum chloride condensation of naphthalene with a chlorinated paraffin wax having preferably 20% to 30% of chlorine, which is substantially higher than the chlorine content of the chlorinated paraffin wax used for the condensation mentioned for stabilizer A, the condensation in this instance being carried out in the presence of a chlorinated hydrocarbon sol-

vent, and the chlorinated paraffin wax being added last to the reaction mixture. The condensation product in this instance not only has pour-depressing properties such as the other materials mentioned above, but also has the property of increasing the viscosity index of a lubricating oil base stock to which it is added.

In preparing the above-described stabilizers, the Friedel-Crafts condensation is preferably carried out in the presence of an inert solvent such as a refined naphtha or kerosene, or tetrachloroethane, and is generally carried out at a temperature between about room temperature and about 300° F., usually being started at room temperature until the initial reaction rate tends to subside and then the reaction mass is heated to a temperature of about 150° F. or 200° F. for about 1-10 hours to insure completion of the reaction, following which the reaction mass is cooled, preferably after dilution with an inert solvent such as refined kerosene. The catalyst is hydrolyzed by adding water, alcohol, aqueous caustic soda, or a mixture of such agents, and after settling or centrifuging, the catalyst layer is removed, and the condensation products, together with solvent or diluent if such were used, are then subjected to distillation, preferably under reduced pressure, such as steam distillation or vacuum distillation under an absolute pressure of about 5-50 mm. of mercury, carrying the distillation up to a temperature of about 500° F. or 600° F., to obtain the desired high molecular weight condensation product as distillation residue. This condensation product has a molecular weight above 500, usually above 1,000, and may range as high as 2,000 or 5,000 or higher. It is generally a dark colored very viscous oily liquid, soluble in mineral oils. If desired, this distillation residue may be subjected to solvent extraction with liquids such as propane, butane, etc., methyl alcohol, etc., ethyl acetate, etc., acetone, etc., in order to obtain a more highly concentrated material as the raffinate. Substantially all of the lower molecular weight materials being removed and leaving a fraction having especially good potency for the stabilizing purposes of the present invention, or for the additional pour-depressing or viscosity index improving properties.

The amount of the stabilizer to be used according to this invention should normally be within the approximate limits of about 0.5% to 15%, preferably about 2% to 10%, about 5% having been found very suitable.

The extreme pressure lubricant to which the above-described stabilizers may be added according to this invention, may be prepared by incorporating into a mineral oil base stock derived from any of the commonly used crude petroleum oils, a compound containing active halogen and a compound containing active sulfur, or one or more compounds containing both halogen and sulfur in the same molecules. The invention is particularly applicable to extreme pressure lubricants containing corrosive chlorine compounds, for instance, chlorinated aliphatic or aromatic hydrocarbons such as chlorinated derivatives of paraffin wax, kerosene, aromatic petroleum fractions, or coal tar solvents. The amount of chlorine, to be used, will of course depend upon the severity of the conditions under which the lubricant is to be used but will generally vary between the approximate limits of 5% and 50% in the chlorinated organic compounds, or between the approximate limits of 1% and 10%

based on the total weight of lubricants. The incorporation of sulfur compounds tends to increase the suitability of the lubricant for use under high temperatures, and the sulfur compounds to be used may be, for instance, sulfurized fatty or mineral oils such as sulfurized sperm oil, or sulfur compounds such as organic sulfides, mercaptans, di- or poly-sulfides, xanthates, xanthogen sulfide, thiocarbonates, thiocyanates, etc. These compounds may be used in such amounts that about 1% to 30% of sulfur is incorporated in the active or combined state, on the basis of the extreme pressure lubricating agent, per se, or about 0.5% to 10% based on the total lubricant.

Instead of using separate chlorine compounds and sulfur compounds, it is possible to use single materials in which both sulfur and halogen have been incorporated. For instance, a suitable raw material such as paraffin wax or a liquid petroleum distillate such as kerosene, may be treated with a sulfur halide such as sulfur mono- or dichloride, in order to incorporate both sulfur and chlorine. A different method and one which is generally preferred commercially because it permits better technical control, is to chlorinate a suitable raw material such as paraffin wax, kerosene, or naphtha, to the desired chlorine content, and then subsequently treat the resultant compound with sulfur or an inorganic sulfide such as sodium sulfide or polysulfide, or a mixture thereof with sulfur and sodium hydroxide, or an organic sulfur compound such as thiocarbonate, xanthate, or thiocyanate.

One example of a suitable extreme pressure lubricating agent is one made by chlorinating kerosene to a chlorine content of about 25% to 50%, such as 35%, by passing chlorine through kerosene at a temperature of about 175° F. to 200° F., and adding to the resultant chlorinated kerosene, an isopropyl alcohol solution of aqueous caustic soda and sodium hydrogen sulfide, containing free sulfur admixed therewith, using a reflux temperature, for a reaction time ranging between about 1/2 hour and 5 or 10 hours. The resultant product may, for instance, contain 7.0% sulfur and 33% chlorine or, as another example, might contain 6.5% sulfur and 31% chlorine. Ordinarily, the stabilizers of this invention will be needed more, and therefore be of greatest advantage, when extreme pressure lubricating agents are used which contain a large amount of sulfur and chlorine.

A compound made by this method and having this latter composition, and marketed under the trade name "Parapoid," will be referred to as "Extreme pressure agent 1," in the tests reported herebelow.

Another example of an extreme pressure lubricating agent which may be used is one made by similiarly chlorinating kerosene to a chlorine content of about 25% to 50%, preferably about 30% to 40%, and treating the resultant chlorinated kerosene with sodium xanthate, as for instance in alcohol solution. The sodium chloride forms and separates out, and the liquid product is distilled free of alcohol, leaving a product, for example, which may contain 9% sulphur and 32% chlorine. A compound marketed under the trade name "Santopoid," and understood to be made by this procedure, will be referred to as "Extreme pressure agent 2" in the tests reported herebelow.

Extreme pressure lubricants made by adding to a lubricating oil base stock separate chlorine and

sulfur compounds may be made by using about 10% by weight of chlorinated paraffin wax containing 40% to 50% of chlorine, and a sulfur compound, such as benzyl disulfide in sufficient amount to impart the desired proportion of sulfur, for instance 1% based on the total lubricant. Instead of using benzyl disulfide, 10% of sulfurized sperm oil containing 10% sulfur, might be used. A product of this type is marketed under the trade name "Anglamol."

The following tests will further explain how the invention is carried out and will also illustrate the advantages of the invention.

An extreme pressure lubricant stability test was devised, which comprised placing 50 cubic centimeters of the extreme pressure lubricating agent to be tested, in a pour test jar capped with a slotted cork. For each set of storage conditions to be studied, two samples of the same material are tested simultaneously, one simply in contact with the glass of the pour jar and the other containing a strip of unpolished boiler plate sheet iron (1" x 2" x 1/4"). As one example of the test storage conditions, the jars are placed

4. Storage in black steel capped pipes under all weather conditions on a building roof, observations being made at 20 and 40 days.

In order to determine whether various chemical compounds or other materials which might be added to the extreme pressure lubricant, would have any stabilizing effect in preventing the deposition of a precipitate or sediment or sludge, during storage, the materials to be tested were added in 5% concentration to the extreme pressure lubricant, and subjected to the stability test described above, adequate control samples being run simultaneously for comparison.

15 Of the numerous materials tested, only a relatively minor proportion had any stabilizing effect in preventing the separation of sediment or sludge during storage, a few materials had no effect at all, and surprisingly, the great majority of the materials tested were accelerators of degradation.

The test results obtained with the materials coming within the scope of the present invention are shown in the following tables.

Table I

*Stability tests after 60 days storage at room temperature*

| Sample                                        | Storage container | Condition <sup>1</sup> of 10% blend in Panhandle B. S. after six days at room temperature |                             |
|-----------------------------------------------|-------------------|-------------------------------------------------------------------------------------------|-----------------------------|
|                                               |                   | Oil layer                                                                                 | Other observations          |
| Extreme pressure agent 1.....                 | Glass.....        | Cloudy.....                                                                               | No sediment present.        |
| Do.....                                       | do.....           | do.....                                                                                   | Slt. amt. sediment present. |
| Extreme pressure agent 1+3% stabilizer A..... | Glass+iron.....   | Slt. cloud.....                                                                           | No sediment present.        |
| Do.....                                       | Glass+iron.....   | do.....                                                                                   | Do.                         |
| Extreme pressure agent 1+6% stabilizer A..... | Glass.....        | do.....                                                                                   | Do.                         |
| Do.....                                       | Glass+iron.....   | do.....                                                                                   | Do.                         |

<sup>1</sup> Observations are made in a 4 oz. oil sample bottle.

TABLE II

*Stability tests after 60 days storage at 120° F.*

| Sample                                        | Storage container | Condition <sup>1</sup> of 10% blend in Panhandle B. S. after six days at room temperature |                             |
|-----------------------------------------------|-------------------|-------------------------------------------------------------------------------------------|-----------------------------|
|                                               |                   | Oil layer                                                                                 | Other observations          |
| Extreme pressure agent 1.....                 | Glass.....        | Cloudy.....                                                                               | No sediment present.        |
| Do.....                                       | Glass+iron.....   | do.....                                                                                   | Slt. amt. sediment present. |
| Extreme pressure agent 1+3% stabilizer A..... | Glass.....        | do.....                                                                                   | No sediment present.        |
| Do.....                                       | Glass+iron.....   | do.....                                                                                   | Do.                         |
| Extreme pressure agent 1+6% stabilizer A..... | Glass.....        | Slt. cloud.....                                                                           | Do.                         |
| Do.....                                       | Glass+iron.....   | do.....                                                                                   | Do.                         |

<sup>1</sup> Observations are made in a 4 oz. oil sample bottle.

in an oven thermostatically controlled at 150° F. for 24 hours, then removed and allowed to cool to room temperature. Degradation in solubility is then determined by making a 10% (by weight) blend of each material in a heavy paraffinic oil such as Panhandle Bright Stock (always using the same material for comparative results), observations being made after 5 to 10 days in order to overcome the initial effect of the blending operation. In the series of tests reported herewith, four different test storage conditions were used, as follows:

1. Storage at room temperature in glass and in the presence of iron, respectively.

2. Storage at 120° F. for 60 days, observations being made at 20, 40, and 60 days.

3. Storage at 150° F. for periods of 24, 48, and 120 hours in glass and in the presence of iron.

60 65 70 75 75  
TABLE III  
*Stability tests after 40 days storage under weather conditions in iron pipe on roof of building*

| Sample                                        | Condition <sup>1</sup> of 10% blend in Panhandle Bright Stock after six days at room temperature |                                                            |
|-----------------------------------------------|--------------------------------------------------------------------------------------------------|------------------------------------------------------------|
|                                               | Oil layer                                                                                        | Other observations                                         |
| Extreme pressure agent 1.....                 | Cloudy.....                                                                                      | Slight amount of sediment present.                         |
| Extreme pressure agent 1+3% stabilizer A..... | do.....                                                                                          | Some scale and water present <sup>2</sup> but no sediment. |
| Extreme pressure agent 1+6% stabilizer A..... | Slt. cloud.....                                                                                  | Do.                                                        |

<sup>1</sup> Observations are made in a 4 oz. oil sample bottle.

<sup>2</sup> Water is due to leakage of pipes during rainfall.

TABLE IV

Storage stability tests at 150° F.

| Sample                                   | Storage container | Time of storage, hours | Condition <sup>1</sup> of 10% blend in Panhandle B. S. after 5 days at room temperature |                                       |
|------------------------------------------|-------------------|------------------------|-----------------------------------------------------------------------------------------|---------------------------------------|
|                                          |                   |                        | Oil layer                                                                               | Other observations                    |
| Extreme pressure agent 1                 | Glass             | 24                     | Cloudy                                                                                  | Sediment present.                     |
| Extreme pressure agent 1+3% stabilizer A | do                | 24                     | do                                                                                      | Sit. sediment present.                |
| Extreme pressure agent 1+6% stabilizer A | do                | 24                     | do                                                                                      | Do.                                   |
| Extreme pressure agent 1                 | Glass+iron        | 24                     | do                                                                                      | 1/4-inch sediment present.            |
| Extreme pressure agent 1+3% stabilizer A | do                | 24                     | do                                                                                      | No sediment present.                  |
| Extreme pressure agent 1+6% stabilizer A | do                | 24                     | do                                                                                      | Sit. amt. sediment present.           |
| Extreme pressure agent 1                 | Glass             | 48                     | do                                                                                      | 1/4-inch sediment present.            |
| Extreme pressure agent 1+3% stabilizer A | do                | 48                     | do                                                                                      | Thin slurry <sup>2</sup> of sediment. |
| Extreme pressure agent 1+6% stabilizer A | do                | 48                     | do                                                                                      | 1/4-inch sediment present.            |
| Extreme pressure agent 1                 | Glass+iron        | 48                     | do                                                                                      | Heavy dispersion <sup>3</sup> .       |
| Extreme pressure agent 1+3% stabilizer A | do                | 48                     | do                                                                                      | Do.                                   |
| Extreme pressure agent 1+6% stabilizer A | Glass             | 120                    | do                                                                                      | 1 1/4 inches sediment present.        |
| Extreme pressure agent 1                 | do                | 120                    | do                                                                                      | Thin slurry <sup>2</sup> of sediment. |
| Extreme pressure agent 1+3% stabilizer A | do                | 120                    | do                                                                                      | 1/4-inch sediment present.            |
| Extreme pressure agent 1+6% stabilizer A | Glass+iron        | 120                    | do                                                                                      | Very heavy sediment present.          |
| Extreme pressure agent 1                 | do                | 120                    | do                                                                                      | 1/4-inch sediment present.            |
| Extreme pressure agent 1+3% stabilizer A | do                | 120                    | do                                                                                      | 1/4-inch sediment present.            |
| Extreme pressure agent 1+6% stabilizer A | do                | 120                    | do                                                                                      | 1/4-inch sediment present.            |

<sup>1</sup> Observations are made if possible from a 4 oz. oil sample bottle.<sup>2</sup> Measurements on the sediment refer to an accumulation on the bottom of the bottle.<sup>3</sup> A dispersion or slurry refers to particle formation which is not extensive enough, or the particles are too fine to settle in 5 days.

TABLE V

Stability tests of extreme pressure lubricants made with 90% of Bright Stock, after 60 hours storage

| Remaining 10% composition (other than 90% Panhandle Bright Stock) | Storage container | Temp. of storage | Condition of expes lube after test |                                      |
|-------------------------------------------------------------------|-------------------|------------------|------------------------------------|--------------------------------------|
|                                                                   |                   |                  | Oil layer                          | Other observations                   |
| 10% extreme pressure agent 1                                      | Glass             | Room             | Heavy cloud                        | Precip. material on sides of bottle. |
| 9.4% extreme pressure agent 1+0.6% stabilizer A                   | do                | do               | Cloudy                             | Very slight amount of sediment.      |
| 10% extreme pressure agent 1                                      | do                | 150° F.          | Clear                              | Slight amount of sediment present.   |
| 9.4% extreme pressure agent 1+0.6% stabilizer A                   | Glass+iron        | 150° F.          | do                                 | No sediment present.                 |
| 10% extreme pressure agent 1                                      | do                | 150° F.          | do                                 | Slight amount of sediment present.   |
| 9.4% extreme pressure agent 1+0.6% stabilizer A                   | do                | 150° F.          | do                                 | No sediment present.                 |

The above tables show that stabilizer A was very effective in stabilizing the extreme pressure agent, as well as the lubricant made therewith, against development and settling out of an insoluble precipitate or sludge during storage under various conditions.

Many other tests were made, and it was found that the materials described hereinabove and referred to as stabilizers B, C, and D are all very effective in stabilizing Extreme pressure agent 1 as well as 10% blends thereof in the Panhandle Bright Stock.

These stabilizers A, B, C, and D may also be used satisfactorily and advantageously in Extreme pressure agent 2 as well as in blends thereof in a mineral oil base stock.

Although the theory as to the exact mechanism of the operation of the invention is not well understood, it is believed that the stabilizer of this invention tends to prevent a self-polymerization of the extreme pressure agent to a heavier and insoluble form during storage. The extreme pressure agent may selectively react with the stabilizer to form a soluble but still effective extreme pressure molecule, rather than reacting with itself to form a higher molecular weight insoluble product.

In preparing extreme pressure lubricants according to this invention, other known addition agents may be incorporated if desired, for instance, fatty oils, soaps of fatty acids or naphthenic acid, other materials having thickening, viscosity-index improving and pour-depressing

properties, anti-oxidants, oil-soluble metal soaps, dyes, etc.

45 It is not intended that this invention be limited to any of the particular examples which have been given merely for illustration, nor by any theory as to the mechanism of the operation of the invention, but only by the appended claims in which it is intended to claim all novelty inherent in the invention as well as other modifications coming within the scope and spirit of the invention.

We claim:

55 1. An extreme pressure lubricating agent containing about 5% to 50% of chlorine and about 1% to 30% of sulfur, and derived by chlorinating a petroleum hydrocarbon fraction and treating the resultant chlorinated hydrocarbon material with a sulfurizing agent, to which has been added a small amount of a condensation product of an aromatic compound and a long aliphatic compound containing a reactive group, said condensation product having a molecular weight above 600, being substantially non-volatile at temperatures up to about 600° F., and being soluble in mineral oil.

70 2. Product according to claim 1, in which the extreme pressure agent contains about 5% to 10% of sulfur and about 25% to 40% of chlorine, and is made by chlorinating kerosene and treating the resultant chlorinated kerosene with a sodium polysulfide sulfurizing agent.

75 3. An extreme pressure lubricant comprising about 90% of a mineral lubricating oil base stock,

and about 10% of an extreme pressure agent containing about 5% to 10% of sulfur, about 25% to 40% of chlorine and obtained by chlorinating kerosene and treating the resultant chlorinated kerosene with sodium polysulfide as the sulfurizing agent, into which extreme pressure lubricant has been incorporated a small amount of a stabilizer against insolubilizing degradation comprising a condensation product of naphtha-

lene with chlorinated paraffin wax containing about 10% to 15% of chlorine, said condensation product having a molecular weight above 1,000, being substantially non-volatile at temperatures up to about 600° F. under reduced pressure, and being soluble in mineral oil.

EUGENE LIEBER.  
ALOYSIUS F. CASHMAN.